

## UNITED STATES PATENT OFFICE

2,666,703

## SINGLE-POWDER PHOTOGRAPHIC DEVELOPERS STABILIZED WITH METABORIC ACID

Donald J. Kridel and Edwin S. Wiitala, Rochester, N. Y., assignors to Eastman Kodak Company, Rochester, N. Y., a corporation of New Jersey

No Drawing. Application June 26, 1952,  
Serial No. 295,834

7 Claims. (Cl. 95—88)

1

This invention relates to single-powder photographic developers, and more particularly to a single-powder developer in which the ingredients of the developer are intimately mixed in the form of dry powder with powdered metaboric acid ( $HBO_2$ ), as a stabilizing agent to prevent disadvantageous interaction between the organic developer component and the basic component of the single-powder mixture.

Heretofore single powder developer mixtures have been prepared and packaged which contain an organic silver halide developer component or mixtures of such components, including monomethyl p-aminophenol sulfate (elon or metol), hydroquinone, p-aminophenol hydrochloride, p-aminophenol sulfate, pyrogallol, parahydroxyphenyl glycine, catechol, diaminophenol hydrochloride, and others, with an alkali component, a stabilizing component, an oxidizing preventer and an antifogging component. The alkali component may be the stable hydrate of an alkali carbonate, a desiccated alkali carbonate, an alkali metaborate, or an alkali sulfite. Generally the stable alkali carbonate monohydrate is preferred. The oxidation preventing compound may be potassium bromide or iodide. Stabilizing components for such a single-powder developer are disclosed in Patent 2,384,592, of September 11, 1945, and include maleic anhydride, salicylic acid, alkali metabisulfite, benzoic anhydride, orthobenzoic sulfimide, phthalimide, and phthalic anhydride. The latter has outstanding stabilizing properties particularly in the presence of either sodium carbonate or borax and has been employed considerably more than the other stabilizers mentioned in the patent.

While the stabilizing effect of the phthalic anhydride is very good, it has been employed most successfully in developer compositions having as the alkali component either sodium carbonate or sodium sulfite, or mixtures thereof. Less success has been attained in the case of the important class of developers containing sodium metaborate as the alkali ingredient. Also the presence of phthalic anhydride in the single-powder developer involves other considerations which are not too desirable. In the first place phthalic anhydride is slowly soluble in water. But the greatest disadvantage of employing phthalic anhydride in single-powder developer mixtures, which contain alkali carbonates and sulfite, is that phthalic anhydride may react due in part to temperature effects with these basic substances and form gas under sufficient pressure to dislodge the hermetically sealed can in which the

2

developer powder is packaged, and often cause a portion of the powder to be ejected with some violence as the package is opened.

An object, therefore, of the present invention is to provide an improved stabilizing agent for single-powder developers.

Another object of the invention is to provide an improved stabilizing agent for single-powder developers which does not possess the disadvantages caused by employment of phthalic anhydride as the stabilizing agent.

A further object of the invention is to provide an improved stabilizing agent which makes possible the production of single-powder developers having improved stabilizing characteristics containing as the alkali ingredient, sodium metaborate.

In accordance with the present invention these and other objects are attained by employing metaboric acid ( $HBO_2$ ) as the stabilizer, instead of other previously known stabilizers, in such single-powder developers which contain both organic developer components and basic components.

25 We have found that metaboric acid does not have the objectionable characteristics possessed by phthalic anhydride. Because metaboric acid is less acid than phthalic anhydride it does not react as easily or as violently as phthalic anhydride with alkali carbonates or alkali sulfites such as sodium carbonate and sodium sulfite. In this respect it is noted that the pH of phthalic anhydride is about 2.4 while the pH of metaboric acid is about 5.4 at 3% concentrations. Metaboric acid is especially suited as a stabilizer and has characteristics required for a stabilizer. It is acidic, relatively colorless, odorless, and stable and has no deleterious action photographically.

A preferred embodiment of the present invention involves the use in the single-powder photographic developer mixture of either the stable hydrate of an alkali carbonate or also a desiccated alkali carbonate. The alkali carbonate hydrate appears to be more stable in the presence of an organic developer than a comparable quantity of the corresponding desiccated alkali carbonate.

The ingredients of a preferred single-powder developer composition may therefore consist of an organic developing agent, such as monomethyl p-aminophenol sulfate, hydroquinone, p-aminophenol hydrochloride, p-aminophenol sulfate, pyrogallol, p-hydroxyphenyl glycine, catechol, diaminophenol hydrochloride, and suitable mixtures thereof, a stable alkali carbonate, such

as sodium carbonate monohydrate; and metaboric acid, and may contain the other well known ingredients normally present in a developer, such as sodium sulfite and potassium bromide, the normal and known function of the alkali sulfite being that of preservative, lessening the oxidation in solution of the organic developing agent; while the known function of potassium bromide is that of a restrainer particularly inhibiting "fog" formation in the development of the silver image. If sodium metaborate is employed its moisture content should be not more than 35% and preferably be about 15%.

In compounding the developer mixture, one may proceed by first mixing the stabilizer and the basic component, adding and mixing therewith the developing agent, which is followed by incorporating the other ingredients. However, one can mix all the ingredients together at the same time without causing any difficulty.

The following examples will serve further to illustrate developer mixtures within the scope of the invention and will also indicate the proportionate quantities in which the respective components can be mixed together in a dry form to make up such single-powder photographic developer mixtures.

*Example 1*

|                                          | Grams |
|------------------------------------------|-------|
| Elon (monomethyl p-amino phenol sulfate) | 3.1   |
| Anhydrous sodium sulfite                 | 45.0  |
| Hydroquinone                             | 12.0  |
| Sodium carbonate monohydrate             | 81.3  |
| Potassium bromide                        | 1.9   |
| Metaboric acid                           | 4.2   |

*Example 2*

|                              | Grams |
|------------------------------|-------|
| Elon                         | 1.5   |
| Anhydrous sodium sulfite     | 22.5  |
| Hydroquinone                 | 6.3   |
| Sodium carbonate, desiccated | 15.0  |
| Potassium bromide            | 1.5   |
| Metaboric acid               | 1.0   |

*Example 3*

|                              | Grams |
|------------------------------|-------|
| Elon                         | 2.2   |
| Anhydrous sodium sulfite     | 96.0  |
| Hydroquinone                 | 8.8   |
| Sodium carbonate monohydrate | 57.5  |
| Potassium bromide            | 5.0   |
| Metaboric acid               | 3.4   |

*Example 4*

|                                          | Grams |
|------------------------------------------|-------|
| Elon                                     | 2.5   |
| Anhydrous sodium sulfite                 | 30.0  |
| Hydroquinone                             | 2.5   |
| Sodium metaborate (10% H <sub>2</sub> O) | 10.5  |
| Potassium bromide                        | 0.5   |
| Metaboric acid                           | 4.7   |

*Example 5*

|                              | Grams |
|------------------------------|-------|
| Sodium sulfite               | 50    |
| Sodium carbonate monohydrate | 54    |
| Potassium bromide            | 1     |
| Metaboric acid               | 2.2   |
| Pyrogallol                   | 6.3   |

*Example 6*

|                              | Grams |
|------------------------------|-------|
| Sodium sulfite               | 50    |
| Sodium carbonate monohydrate | 54    |
| Potassium bromide            | 1     |
| Metaboric acid               | 2.2   |
| Catechol                     | 5.5   |

*Example 7*

|                              | Grams |
|------------------------------|-------|
| Sodium sulfite               | 50    |
| Sodium carbonate monohydrate | 54    |
| Potassium bromide            | 1     |
| Metaboric acid               | 2.2   |
| p-Hydroxyphenyl glycine      | 8.4   |

*Example 8*

|                              | Grams |
|------------------------------|-------|
| Sodium sulfite               | 50    |
| Sodium carbonate monohydrate | 54    |
| Potassium bromide            | 1     |
| Metaboric acid               | 2.2   |
| p-Aminophenol sulfate        | 7.3   |

*Example 9*

|                              | Grams |
|------------------------------|-------|
| Sodium sulfite               | 50    |
| Sodium carbonate monohydrate | 54    |
| Potassium bromide            | 1     |
| Metaboric acid               | 2.2   |
| p-Aminophenol hydrochloride  | 7.3   |

*Example 10*

|                              | Grams |
|------------------------------|-------|
| Sodium sulfite               | 75    |
| Sodium carbonate monohydrate | 30    |
| Potassium iodide             | .01   |
| Metaboric acid               | 2.2   |
| Hydroquinone                 | 9     |
| Elon                         | 1     |

*Example 11*

|                          | Grams |
|--------------------------|-------|
| Elon                     | 10.0  |
| Anhydrous sodium sulfite | 100.0 |
| Sodium metaborate        | 20.0  |
| Metaboric acid           | 4.0   |

*Example 12*

|                            | Grams |
|----------------------------|-------|
| Elon                       | 7.5   |
| Sodium sulfite, desiccated | 100.0 |
| Metaboric acid             | 1.1   |

*Example 13*

|                              | Grams |
|------------------------------|-------|
| Sodium sulfite               | 96    |
| Sodium carbonate monohydrate | 56    |
| Potassium bromide            | 5     |
| Metaboric acid               | 1.7   |
| Hydroquinone                 | 8.8   |
| Elon                         | 2.2   |

*Example 14*

|                             | Grams |
|-----------------------------|-------|
| Diaminophenol hydrochloride | 34.6  |
| Sodium sulfite              | 59.2  |
| Potassium bromide           | 3.2   |
| Metaboric acid              | 2.9   |

*Example 15*

|                              | Grams |
|------------------------------|-------|
| Elon                         | 3.0   |
| Sodium sulfite               | 45.0  |
| Hydroquinone                 | 12.0  |
| Sodium carbonate monohydrate | 80.0  |
| Potassium bromide            | 0.6   |
| 5-methyl benzotriazole       | 0.06  |
| Metaboric acid               | 1.4   |

In preparing a developer solution the compositions of the above examples should be dissolved in water to make one liter of solution.

Samples of the powders stabilized with metaboric acid as given in the examples have been found, even after they have been kept in hermetically sealed cans at 120° F. for prolonged periods, to be unimpaired in developing proper-

## 5

ties and to give a solution comparable in color to solutions prepared from such chemicals not previously mixed. No expansion of the package in which the compositions were stored was noted as contrasted to the developers similar in composition except that phthalic anhydride replaces the metaboric acid of the present invention.

We claim:

1. A stable single-powder photographic developer composition containing an organic silver halide developer, a stabilizing agent comprising metaboric acid and a soluble, stable, and photographically compatible basic ingredient selected from the group consisting of alkali borates, sulfites and carbonates.

2. A stable single-powder photographic developer composition containing an organic silver halide developer, a stabilizing agent comprising metaboric acid, an antifoggant, and a soluble, stable, and photographically compatible basic ingredient selected from the group consisting of alkali borates, sulfites and carbonates.

3. A stable single-powder photographic developer composition containing an organic silver halide developer, sodium carbonate monohydrate, and metaboric acid.

## 6

4. A stable single-powder photographic developer containing an organic silver halide developer, alkali carbonate, an alkali sulfite and metaboric acid.

5. A stable single-powder photographic developer containing an organic silver halide developer, an anhydrous alkali carbonate, an alkali sulfite and metaboric acid.

6. A stable single-powder photographic developer composition containing an organic silver halide developer, sodium sulfite, sodium metaborate, and metaboric acid.

7. A stable single-powder photographic developer composition containing an organic silver halide developer 5-methyl benzotriazole and metaboric acid.

DONALD J. KRIDEL.  
EDWIN S. WIITALA.

## References Cited in the file of this patent

## UNITED STATES PATENTS

| Number    | Name   | Date         |
|-----------|--------|--------------|
| 2,606,118 | Rogers | Aug. 5, 1952 |